

## 1

2,938,789

TITANIUM-MOLYBDENUM ALLOYS WITH  
COMPOUND FORMERS

Robert I. Jaffee, Columbus, Ohio, assignor, by mesne assignments, to Kennecott Copper Corporation, New York, N.Y., a corporation of New York

No Drawing. Filed May 18, 1959, Ser. No. 813,619

4 Claims. (Cl. 75—175.5)

This invention relates to ternary and more complex alloys containing titanium and molybdenum and particularly to titanium alloys, in which molybdenum is a major alloying element, which exhibit superior mechanical and chemical properties.

This application is a continuation-in-part of copending application Serial No. 509,490, filed May 19, 1955, now abandoned.

Titanium metal and titanium alloys are light, relatively strong metals and are in great demand today as preferred materials for use in aircraft and jet engines, as well as other applications where light and strong materials are needed. There is a continual effort to improve the mechanical and chemical properties of titanium in order to satisfy the demands for light metals with high-strength and corrosion-resistance properties.

Important strides have been taken in obtaining superior corrosion-resistance and mechanical properties by alloying titanium with molybdenum. Titanium alloys containing less than 40 percent molybdenum are well known. These alloys have excellent hardness and strength. Titanium-base alloys containing more than 45 percent molybdenum have little value commercially, in that they are difficult to work even at elevated temperatures and thus are difficult to produce in the wrought condition for subsequent fabrication. Titanium alloys containing less than 30 percent molybdenum are of less value, in that their strength and hardness are not as great as those containing 30 percent molybdenum or more.

The improvement of mechanical or corrosion-resistant properties is of great significance in the search for strong, light metals.

It has not been discovered that very desirable properties can be imparted to titanium-molybdenum alloys by further alloying with certain elements to form ternary and even more complex alloys.

In the titanium-molybdenum system, an increase in strength without a decrease in workability is a highly significant development.

It is, therefore, an object of this invention to improve the properties of titanium by alloying with molybdenum plus certain ternary additions and combinations thereof.

It is another object of this invention to provide complex alloys containing titanium and molybdenum that are workable and that possess high strength at both room temperature and elevated temperatures.

It is a further object of this invention to provide ternary alloys containing titanium and molybdenum that possess superior mechanical properties as compared to titanium, and titanium-molybdenum binary alloys.

It is also an object to provide alloying additions suitable for replacing molybdenum and titanium in titanium-molybdenum alloys.

## 2

Other objects and advantageous features of this invention will be obvious from the following specification.

In general, this invention relates to high-strength complex alloys in which titanium and molybdenum are major constituents. Titanium-molybdenum ternary alloys containing at least one compound-forming addition selected from the group consisting of boron and silicon have been found to have superior strength to titanium and to titanium-molybdenum binary alloys with equivalent molybdenum contents. In addition, such ternary alloys have superior workability to titanium-molybdenum binary alloys at the 50 percent molybdenum level.

Titanium-molybdenum alloys containing ternary additions, selected from the group of compound-forming additions, which have limited solubilities in both alpha and beta titanium, have also been found to have superior strength properties. These ternary additions also greatly improve the workability of the titanium, 50-percent-molybdenum alloy. As has been stated, titanium alloys containing more than 45 percent molybdenum are difficult to work, even at high temperatures. Titanium-molybdenum alloys containing as much as 50 percent molybdenum were successfully hot-rolled or worked when small additions (up to 2 percent) of boron or silicon were made. Table I below lists the compound-forming additions and gives the preferred minimum and maximum amounts of each alloying constituent in the ternary ranges.

Table I

| Element      | Ternary Addition |      | Molybdenum, Percent |      | Titanium, Percent |      |
|--------------|------------------|------|---------------------|------|-------------------|------|
|              | Percent          |      | Min.                | Max. | Min.              | Max. |
|              | Min.             | Max. |                     |      |                   |      |
| Boron.....   | 0.1              | 1.0  | 30                  | 50   | 50                | 70   |
| Silicon..... | 0.1              | 2.0  | 30                  | 50   | 50                | 70   |

It is obvious that additions of boron and silicon can be made to ternary alloys of titanium and molybdenum for the purpose of improving their workability. In particular it has been found that high-strength titanium-molybdenum alloys consisting essentially of from 30 to 50 percent molybdenum together with up to 20 percent of a beta stabilizing metal are improved as to workability by the addition of at least one titanium compound former from the group consisting of boron and silicon in amounts from 0.1 to 2.0 percent. Well known beta stabilizers for these alloys include columbium, tantalum, tungsten, and chromium.

As can be seen in Table II the above-described alloys exhibit far superior mechanical properties to unalloyed titanium and have a strengthening effect on the titanium-molybdenum binary alloys with equivalent molybdenum contents.

The ternary and complex alloys of the present invention are highly corrosion resistant in both acid and basic media. In an attempt to develop the grain structure of the alloys, a total of 13 acid and 2 basic etching solutions were used at a temperature of 75° F. Also, samples were exposed to concentrated sulfuric and 25 weight percent potassium hydroxide at 170° F. None of these etchants produced grain boundary attack.

The following table covering nearly all of the ranges disclosed above is presented to more clearly illustrate the effects of the alloy additions of this invention.

Table II

| Composition, Weight Percent (Balance Ti) | Rollability <sup>1</sup> | Vickers Hardness Number |        |         |         |         | Yield Strength, p.s.i.—0.2% Offset | Ultimate Tensile Strength, p.s.i. | Total Elongation, Percent | Reduction in Area, Percent | Bend Ductility, T Value <sup>2</sup> |  |  |  |  |  |
|------------------------------------------|--------------------------|-------------------------|--------|---------|---------|---------|------------------------------------|-----------------------------------|---------------------------|----------------------------|--------------------------------------|--|--|--|--|--|
|                                          |                          | Wrought                 |        |         |         |         |                                    |                                   |                           |                            |                                      |  |  |  |  |  |
|                                          |                          | Cast, 25° C.            | 25° C. | 500° C. | 700° C. | 900° C. |                                    |                                   |                           |                            |                                      |  |  |  |  |  |
| Unalloyed.....                           | Rollable.....            | 161                     | 176    | 61      | <25     | <20     | 47,500                             | 67,100                            | 31                        | 53                         | 0.0                                  |  |  |  |  |  |
| <b>Ti-Mo ALLOYS</b>                      |                          |                         |        |         |         |         |                                    |                                   |                           |                            |                                      |  |  |  |  |  |
| 30 Mo.....                               | Rollable.....            | 253                     | 246    | 186     | 118     | 52      | 110,500                            | 115,100                           | 13                        | 31                         | 1.1                                  |  |  |  |  |  |
| 35 Mo.....                               | do.....                  | 271                     | 262    | 221     | 182     | 66      | 121,400                            | 121,400                           | 7                         | 24                         | 2.2                                  |  |  |  |  |  |
| 40 Mo.....                               | do.....                  | 291                     | 283    | 211     | 161     | 76      | 131,600                            | 132,500                           | 2                         | 11                         | 3.4                                  |  |  |  |  |  |
| 45 Mo.....                               | do.....                  | 331                     | 290    | 208     | 173     | 84      | 140,800                            | 143,200                           | 1                         | 11                         | —                                    |  |  |  |  |  |
| 50 Mo.....                               | Not Rollable.....        | 315                     | 328    | 254     | 221     | 159     |                                    |                                   |                           |                            |                                      |  |  |  |  |  |
| <b>Ti-Mo-B ALLOYS</b>                    |                          |                         |        |         |         |         |                                    |                                   |                           |                            |                                      |  |  |  |  |  |
| 30 Mo, 0.1 B.....                        | Rollable.....            | 261                     | 250    | 174     | 93      | 53      | 115,800                            | 117,700                           | 12                        | —                          | 1.3                                  |  |  |  |  |  |
| 30 Mo, 0.5 B.....                        | do.....                  | 292                     | 274    | 178     | 110     | 52      | 123,200                            | 128,300                           | 11                        | —                          | 1.9                                  |  |  |  |  |  |
| 40 Mo, 0.1 B.....                        | do.....                  | 269                     | 278    | 218     | 156     | 72      | 125,400                            | 131,100                           | 5                         | —                          | 5.4                                  |  |  |  |  |  |
| 50 Mo, 0.1 B.....                        | do.....                  | 336                     | 325    | 244     | 217     | 161     | Brittle Fracture                   |                                   | <1                        | —                          | >18.2                                |  |  |  |  |  |
| <b>Ti-Mo-Si ALLOYS</b>                   |                          |                         |        |         |         |         |                                    |                                   |                           |                            |                                      |  |  |  |  |  |
| 30 Mo, 0.5 Si.....                       | Rollable.....            | 288                     | 281    | 171     | 112     | 33      | 125,000                            | 128,900                           | 7                         | —                          | 1.3                                  |  |  |  |  |  |
| 30 Mo, 1.0 Si.....                       | do.....                  | 239                     | 258    | —       | 106     | 23      | 120,200                            | 125,100                           | 11                        | —                          | 1.6                                  |  |  |  |  |  |
| 40 Mo, 0.5 Si.....                       | do.....                  | 321                     | 319    | 256     | 192     | 78      | Brittle Fracture                   |                                   | <1                        | —                          | 15.6                                 |  |  |  |  |  |
| 50 Mo, 0.5 Si.....                       | do.....                  | 347                     | 365    | 286     | 244     | 134     |                                    |                                   |                           | —                          | >22.0                                |  |  |  |  |  |

<sup>1</sup> Pack rolled in mild steel sheath at 900° C.<sup>2</sup> T Value—minimum satisfactory bend radius divided by the specimen thickness.

What is claimed is:

1. A high-strength alloy in which titanium is a major constituent and consisting essentially of from about 30 to 50 percent molybdenum, from about 0.1 to 2.0 percent of at least one titanium compound-forming addition selected from the group consisting of boron and silicon, balance titanium, said alloy being characterized by superior workability as compared with that of titanium-molybdenum alloys of comparable molybdenum content.

2. A high-strength alloy in which titanium is a major constituent consisting essentially of from 30 to 50 percent molybdenum, and from .1 to 1.0 percent boron, and characterized by high workability as compared to titanium-molybdenum binary alloys in the same molybdenum range.

3. A high-strength alloy in which titanium is a major constituent consisting essentially of from 30 to 50 percent molybdenum, and from .1 to 2 percent silicon, and characterized by high workability as compared to titanium-molybdenum binary alloys in the same molybdenum range.

4. The method of improving the workability of titanium-molybdenum alloys containing molybdenum in the range from 30 to 50 percent, comprising the step of alloying at least one compound-forming addition selected from the group consisting of boron in an amount ranging from 0.1 to 1.0 percent, and silicon in an amount ranging from 0.1 to 2.0 percent with said titanium-molybdenum alloys.

40

## References Cited in the file of this patent

## UNITED STATES PATENTS

|           |               |               |
|-----------|---------------|---------------|
| 2,614,041 | Finlay        | Oct. 14, 1952 |
| 2,818,333 | Swazy et al.  | Dec. 31, 1957 |
| 2,819,960 | Bomberger     | Jan. 14, 1958 |
| 2,821,475 | Jaffee et al. | Jan. 28, 1958 |
| 2,893,864 | Harris et al. | July 7, 1959  |

## OTHER REFERENCES

Transactions, AIME, April 1951, pages 335-336, article by Ogden and Jaffee.

"Titanium-Silicon Alloys," Metal Treatment and Drop Forging, April 1954, pages 191-197.

50